

(No Model.)

D. TORREY.

Pile for the Manufacture of Composite Plates.

No. 235,471.

Patented Dec. 14, 1880.

Fig. 1.



Fig. 2.



WITNESSES:

*A. Schekl*  
*C. Sedgwick*

INVENTOR:

*D. Torrey*  
BY *Murphy & Co.*  
ATTORNEYS.

# UNITED STATES PATENT OFFICE.

DOLPHUS TORREY, OF NEW YORK, N. Y.

## PILE FOR THE MANUFACTURE OF COMPOSITE PLATES.

SPECIFICATION forming part of Letters Patent No. 238,471, dated December 14, 1880.

Application filed April 22, 1880. (No model.)

*To all whom it may concern*

Be it known that I, DOLPHUS TORREY, of the city, county, and State of New York, have invented a new and Improved Pile of Iron and Steel for the Manufacture of Composite Plates or Bars, of which the following is a specification.

This invention relates to the protection of the metal forming the interior of the pile from the action of oxidizing flames and gases while in the heating-furnace and immediately subsequent thereto.

The object of my invention is to so shape the pieces of metal forming the box or case of the pile that no bands, ties, bolts, or rivets will be required to keep the separate pieces in proper position.

Figure 1 is a perspective view of the pile with the top removed. Fig. 2 is a perspective view of a pile complete.

Similar letters of reference indicate corresponding parts.

In the drawings, A represents the iron bottom of the pile. B represents the iron top of the pile. C represents the iron band forming the sides of the pile, and D represents the pieces of metal forming the interior of the pile.

Heretofore piles for similar purposes have been made by constructing their cases of separate pieces of iron, usually six in number, which required the use of bands, ties, bolts, or rivets to keep them in position on or around the pile. Such provisions for incasing the interior mass of metal are, however, expensive, troublesome to apply, and often detrimental to the product.

By the method of piling herein shown and described the objectionable features of ordinary piling are avoided, and the two metals (iron and steel) may be simultaneously brought to a welding-heat, and in this condition subjected to the rolls or hammer; and in this form of pile oxygen is practically excluded from the contained steel while in the furnace and during the subsequent manipulations.

In the heating of this pile in the furnace a chemical action takes place similar to that which occurs in the manufacture of blister-steel—namely, the combination of a portion of the carbon from the steel with the incasing iron, so that the surfaces of the iron and the steel that are in contact with each other are alike converted into a steely iron or weld-steel, that permits the perfect welding of the parts together when the pile is being formed into plates or bars.

I am aware that it is not new to make a box-pile with its sides and one end in a single piece; but being open at the end access is furnished to the furnace-flames, so as to occasion oxidation and consequent loss. Moreover, steel-scrap cannot be worked with a pile like this, because in passing through the rolls at a welding-heat the soft steel would be forced out.

What I claim as new is—

A closed pile consisting of the plates A, B, intermediate band, C, and steel-scrap D, as shown and described.

DOLPHUS TORREY.

Witnesses:

I. I. STORER,  
C. SEDGWICK.